

April 16, 1929.

C. D. MILLER

1,709,033

PYROTECHNIC DEVICE

Filed Nov. 5, 1926



INVENTOR.  
*Charles D. Miller.*

BY

*Ralph Bush*

ATTORNEY.

## UNITED STATES PATENT OFFICE.

CHARLES D. MILLER, OF BERKELEY, CALIFORNIA.

## PYROTECHNIC DEVICE.

Application filed November 5, 1926. Serial No. 146,395.

My invention relates to pyrotechnic devices and more particularly to the type commonly known as sparklers.

It is well known in the art that sparklers are generally formed by coating a metal base with a composition comprising aluminum powder, or other fuel capable of producing a high temperature upon combustion, an oxidizing compound such as a chlorate or 10 nitrate containing large available quantities of oxygen, and iron or steel chips, which mass is ignited with a match or other such heat producing means and it is the primary object of my invention to provide a sparkler 15 having fulminating tip for igniting the sparkler mass without recourse to other auxiliary heat producing means.

A further object of the invention is to provide a sparkler having a friction igniting 20 tip composed of ingredients capable of producing an intense and prolonged heat necessary to ignite the sparkler mass.

Other objects and advantages of the invention will be apparent during the course 25 of the following description.

In the accompanying drawing, forming a part of this specification and in which like numerals are employed to designate like parts throughout the same,

30 Fig. 1, is a longitudinal sectional view of one form of the invention,

Fig. 2, is a similar view of another form of the invention,

35 Fig. 3, is a view of the scratching surface used in conjunction with the form shown in Fig. 2, and,

Fig. 4, is a longitudinal sectional view of another form of the invention.

In the drawing, wherein for the purpose 40 of illustration, I have shown the preferred forms of my invention, the numeral 5 denotes the usual metal base or rod used in the construction of sparklers, coated with a suitable ignitable composition for the greater 45 portion of its length forming the sparkler mass 6, which is ignited when subjected to the proper heat.

Referring more particularly to my invention, the sparkler mass at its upper end is provided with an enlarged head or tip 7 formed of a suitable fulminating composition for producing an intense and prolonged heat sufficient to ignite the sparkler mass.

The composition for my tip in Fig. 1, consists of the following ingredients combined 50 in substantially the proportions stated: two

parts of fine glue; four parts of water; four to five parts potassium chlorate; one and one-half to two parts amorphous phosphorous; three to four parts powdered glass; one and one-half parts manganese dioxide; four parts magnesium or aluminum powder; two parts sulphur flowers and coloring matter such as red lead or the like if desired.

60 The composition is prepared by first mixing the fine glue and water and heating from 200 degrees to 210 degrees Fahrenheit. The other ingredients are then thoroughly mixed with the mass and the composition is applied to the end of the sparkler mass in any suitable 65 manner. This composition provides a tip which will readily ignite when rubbed against any rough surface and in turn will 70 ignite the sparkler mass.

The form of my invention shown in Fig. 2, 75 comprises a composition consisting of the following ingredients combined in substantially the proportions stated: six parts chloride of potash; two to three parts of antimony sulphide; one part of glue; three parts of manganese dioxide; six parts magnesium or 80 aluminum powder. The ingredients are thoroughly mixed to form a paste which is applied to the end of the sparkler in any suitable manner.

85 A scratching or rubbing surface 10 is used in connection with this form of the invention and is composed of a composition consisting of the following ingredients combined in substantially the proportions stated: ten parts amorphous phosphorous; eight parts antimony sulphide or peroxide of manganese; and three to six parts of glue. The ingredients are thoroughly mixed to form a paste which is spread upon a suitable base, as shown in 90 Fig. 3. This method insures a safe tip which will only ignite upon being scratched or rubbed on a surface covered with a composition as set forth above.

95 The form of my invention shown in Fig. 4, 100 consists of a double tip formed in two parts 8 and 9. The composition for the part 8 consists of the following ingredients in substantially the proportions stated; two parts fine glue; four parts water; four to five parts potassium chlorate; four parts magnesium or aluminum powder; two parts manganese dioxide and two parts sulphur flowers. These ingredients are thoroughly mixed to form a 105 paste which is applied directly to the end of the sparkler mass.

The composition for the part 9 of the tip

consists of the following ingredients combined in substantially the proportions stated: three to four parts of powdered glass; two parts fine glue; two parts sulphur flowers; 5 two parts amorphous phosphorus and four to five parts potassium chlorate. The ingredients are thoroughly mixed to form a paste which is applied to the top of the part 8. The part 9 of this form of tip will be 10 ignited upon being scratched or rubbed upon any rough surface and in turn ignites the part 8 which in turn ignites the sparkler mass.

Thus, it is seen that I have provided various forms of fulminating tips for sparklers 15 formed of compositions capable of producing an intense and prolonged heat to ignite the sparkler mass without recourse to matches or other heat producing means.

Having thus described my invention, I 20 claim:—

1. A composition tip for pyrotechnic sparklers consisting of fine glue, water, potassium chlorate, amorphous phosphorus, powdered glass, manganese dioxide, metallic 25 particles, and sulphur flowers.

2. A fulminating tip for pyrotechnic sparklers consisting of two parts of glue, four parts water, four parts potassium chlorate, two parts amorphous phosphorus, four parts 30 powdered glass, one and one-half parts manganese dioxide, four parts metallic particles and two parts sulphur flowers.

3. The combination with a pyrotechnic sparkler composition of a fulminating tip 35 consisting of an inflammable substance including metallic particles capable of being applied directly to the sparkler mass and ignitable by friction.

4. An inflammable composition capable of 40 being applied directly to a sparkler mass composed of glue, water, potassium chlorate, metallic particles, manganese dioxide and sulphur flowers, in combination with the friction igniting tip superimposed upon the inflammable composition composed of powdered glass, fine glue, sulphur flowers, amorphous phosphorus and potassium chlorate. 45

5. A fulminating tip for pyrotechnic sparklers consisting of two parts of glue, four parts water, four parts potassium chlorate, two parts amorphous phosphorus, four parts powdered glass, one and one-half parts manganese dioxide, four parts magnesium and aluminum powder and two parts sulphur flowers. 50

6. The combination with a pyrotechnic sparkler composition of a fulminating tip consisting of an inflammable substance including magnesium and aluminum powder, capable of being applied directly to the sparkler mass and ignitable by friction.

In testimony whereof I affix my signature.

CHARLES D. MILLER.